

# United States Patent Office

2,702,819

Patented Feb. 22, 1955

1

2,702,819

## GUANIDINE ALKYL ARYL SULFONATES

William N. Axe and William B. Whitney, Bartlesville, Okla., assignors to Phillips Petroleum Company, a corporation of Delaware

No Drawing. Application July 23, 1951,  
Serial No. 238,190

21 Claims. (Cl. 260—501)

This invention relates to guanidine sulfonates as new compositions. In one embodiment this invention relates to novel guanidine salts of synthetic alkyl aryl sulfonic acids. In another embodiment this invention relates to guanidine salts of petroleum sulfonic acids as new compositions.

This application is a continuation-in-part of our copending application Serial No. 217,669, filed March 26, 1951, now Patent Number 2,660,562, which is itself a continuation-in-part of our copending application Serial No. 44,575, filed August 16, 1948, now abandoned.

An object of our invention is to provide as new compositions guanidine salts of petroleum sulfonic acids, having especial utility as lube oil detergents, and as gelation agents in the manufacture of greases. Another object is to provide as new compositions guanidine salts of synthetic alkyl aryl sulfonic acids, having especial utility as lube oil detergents, and as gelation agents in the manufacture of greases. Another object is to provide oil-soluble guanidine petroleum sulfonates. Another object is to provide guanidine alkyl aryl sulfonates, having a total of from 10 to 20 carbon atoms in the alkyl groups. Another object is to provide guanidine petroleum sulfonates containing from 20 to 70 carbon atoms in the molecule. Other objects will be apparent to those skilled in the art from the accompanying discussion and disclosure.

Certain of our guanidine alkyl aryl sulfonates are oil-insoluble and disperse readily in mineral oil as gelation agents to form improved greases of the ashless type, while others, of relatively high molecular weight are oil-soluble, and when dissolved in a lube oil base stock impart valuable detergent properties to it thus forming improved lubricating oils. Certain of our guanidine petroleum sulfonates are oil-soluble and when dissolved in a base lube oil stock impart valuable detergent properties to it, while other guanidine petroleum sulfonates differing from the detergent types principally in molecular weight and/or degree of sulfonation, have pronounced activity as gelation agents when dispersed in the oil, and may be utilized to advantage in the preparation of greases.

Our guanidine alkyl aryl sulfonates particularly suitable as grease gelation agents contain from 17 to 35 carbon atoms in the molecule, although those containing from 24 to 34 carbon atoms can serve also as detergents in oil systems, particularly when so utilized in relatively small concentrations in the lubricating oil. Preferably our guanidine alkyl aryl sulfonates when utilized as oil detergents contain from 40 to 70 carbon atoms per molecule or higher. When employing our guanidine petroleum sulfonates as oil detergents we have found that they should contain at least 40 carbon atoms in the molecule generally up to as high as 70. Our guanidine petroleum sulfonates suitable as gelation agents in the manufacture of greases contain more than 20 and up to 40 carbon atoms in the molecule, preferably from 22 to 35. Also, guanidine petroleum di- or poly-sulfonates derived from heavy petroleum fractions containing over about 40 to as high as about 80 or more carbon atoms in the molecule are excellent gelation agents. These latter compositions have such a molecular weight that the molecule contains one sulfonate group per 20 to 25 carbon atoms.

In the utilization of our guanidine petroleum sulfonates or our guanidine alkyl aryl sulfonates as oil detergents, the resulting oil composition contains from 0.1 to as high as 25 weight per cent or higher, as desired, of the oil-soluble guanidine salt. When utilizing our guanidine

2

sulfonate compositions as gel-forming agents in the manufacture of greases, the resulting grease contains generally from 5 to as high as 60 weight per cent of the gelation agent. In general, the "lubricant," which term denotes either a lubricating grease or a lubricating oil incorporated with a guanidine sulfonate of our invention, generally contains from 0.1 to 60 weight per cent of the guanidine sulfonate added.

In accordance with one method of preparing our guanidine alkyl aryl sulfonates, a synthetic alkyl aryl sulfonic acid is neutralized with guanidine or a basic guanidine salt. The synthetic alkyl aryl sulfonic acid can be prepared in any suitable manner. Any suitable alkylation procedure for alkylating an aromatic hydrocarbon with an olefin can be utilized in the formation of the synthetic alkyl aromatic, which can then be sulfonated to produce the desired synthetic alkyl aryl sulfonic acid. In carrying out such an alkylation a catalyst is generally preferred exemplary of which is sulfuric acid, hydrofluoric acid, boron trifluoride, or the like.

Aromatic hydrocarbons from which our guanidine alkyl aryl sulfonates are derived generally contain from 1 to 3 rings in the aromatic nucleus illustrative of which are benzene, naphthalene, diphenyl or anthracene, or their alkyl derivatives.

One specific method of preparing guanidine alkyl aryl sulfonates suitable for use as gelation agents in the manufacture of greases, comprises the steps of alkylating an aromatic hydrocarbon of the type described in the presence of a suitable alkylation catalyst with an olefin or olefin fraction boiling in the range of 190-315° C., the olefin being selected so that the total number of carbon atoms in the alkyl groups does not exceed 20. The resulting aromatic-olefin alkylation product is then sulfonated employing any suitable sulfonation agent, as for example fuming sulfuric acid, sulfur trioxide or the like to produce the alkyl aryl sulfonic acid. The synthetic sulfonic acid thus formed is then dissolved in a low boiling alcohol such as for example isopropyl alcohol to which resulting solution is added a molar excess of guanidine generally as a concentrated aqueous guanidine solution or as a basic guanidine salt as for example aqueous guanidine carbonate. The resulting reaction solution separates into an alcohol layer containing the guanidine alkyl aryl sulfonate. The alcohol layer is then isolated after which the alcohol is evaporated to recover the guanidine alkyl aryl sulfonate product.

In the preparation of guanidine petroleum sulfonates as oil detergents, we prefer to employ a deasphalted and solvent refined bright stock fraction in the sulfonation step, such as a petroleum fraction having a viscosity range between about 80 and 700 SUS at 210° F. Such a petroleum stock particularly preferred for this purpose, i. e., for sulfonation and subsequent neutralization with guanidine, is a propane-fractionated solvent refined dewaxed Mid-Continent oil having a viscosity of from about 200 to 230 SUS at 210° F., and having a viscosity index of about 85-95 or higher. It will be appreciated by those skilled in the art that by the term "propane-fractionated" is meant fractionation of the oil or bright stock with propane to effect deasphaltization and also separation of oil components on basis of viscosity and that by "solvent refining" is meant the removal by solvent extraction of the more highly aromatic fractions from the deasphalted bright stock. In the latter step any suitable selective solvent can be employed, among which are included phenol, cresylic acids, chlorinated ethers such as chloroethyl ether, nitrobenzene, furfural, and the like. The deasphalted and solvent refined oil is generally dewaxed prior to sulfonation although dewaxing can be dispensed with if complete segregation of sulfonic acids from the waxy oil is carried out at temperatures above the solution temperature of the wax. In any case prior deasphalting and extraction is definitely required. In general, lube stocks lighter than about 80 SUS at 210° F. are unsatisfactory for use in the manufacture of our guanidine petroleum sulfonate oil detergents since the guanidine petroleum sulfonates so produced are not sufficiently soluble in oil to serve as detergent additives.

A feature of our success in producing high molecular weight petroleum sulfonic acids, for neutralization with

guanidine to form guanidine petroleum sulfonate detergents, is the employment of stabilized liquid sulfur trioxide as the sulfonating agent. Our procedure for sulfonating with this reagent is well known in the art and involves dissolving the anhydrous liquid  $\text{SO}_3$  in from 2 to 5 times its weight of dry ethylene chloride to provide an easily manipulated sulfonation reagent. The hydrocarbon sulfonation stock may likewise be dissolved in ethylene chloride or any other suitable non-reactive solvent such as carbon tetrachloride, chloroform, pentane, hexane, or the like.

Sulfonation of the hydrocarbon oil can be carried out in a continuous flow system or in batch agitators. In either case we prefer to employ  $\text{SO}_3$  as the sulfonating agent, and the quantity of  $\text{SO}_3$  added is ordinarily adjusted to give a molar ratio of  $\text{SO}_3$  to sulfonation stock of between about 1:1 and 3:1. The reaction between the hydrocarbon and  $\text{SO}_3$ , even in the case of extremely viscous bright stocks having molecular weights in the range of 800 to 900, is very rapid and exothermic. Sulfonation temperatures are ordinarily controlled within the range of about 50 to 200° F. with a preferred operating range between 80 and 130° F. Lower temperatures may be employed without seriously slowing down reaction rates, but no particular advantage accrues therefrom. At temperatures above about 200° F. excessive oxidation with liberation of sulfur dioxide occurs.

On completion of the sulfonation reaction sufficient aqueous guanidine carbonate solution is added to bring both the oil and water phases to a pH value within the range of 6 to 8 as determined on a pH meter. The aqueous phase is separated and water-soluble reaction products such as guanidine sulfate, sulfite, carbonate and certain polysulfonates are washed from the oil phase with water or water containing some isopropyl alcohol if serious emulsion difficulties are encountered. Separation of oil-insoluble and oil-soluble sulfonates is accomplished by extracting the water-washed oil solution and/or dispersion with an anhydrous alcohol. We have found that petroleum sulfonates of poor oil solubility characteristics are more soluble in anhydrous alcohols such as isopropyl alcohol than are the oil-soluble sulfonates. Since the guanidine petroleum sulfonates are strongly surface-active, emulsion formations can be avoided in this extraction step by dissolving the oil-sulfonate mixture in an equal volume of hot alcohol, i. e., above 100° F. and as high as 150° F. or higher, as for example at its boiling point, and then slowly cooling to room temperature, e. g., to below about 100° F. followed by separation of the alcoholic phase. We have found that continuation of this batchwise extraction is desirable until the alcohol extract no longer forms guanidine picrate when treated with alcoholic picric acid. For reasons not clearly understood, detergent-active guanidine petroleum sulfonates do not react with alcoholic picric acid. Ordinarily 3 to 4 extractions using one volume of alcohol per volume of oil per extraction suffices to complete the desired separation. Residual alcohol is stripped from the oil-detergent solution to give a concentrate suitable for direct addition to lubricating oils, or from which the guanidine petroleum sulfonate produced can be recovered if desired, as for example by silica-gel percolation.

The advantages of this invention are illustrated in the following examples. The reactants and their proportions and their specific ingredients are presented as being typical and should not be construed to limit the invention unduly.

#### EXAMPLE I

Toluene was alkylated with dodecene-1 in the presence of a boron trifluoride-water complex as a catalyst. The catalyst was prepared by bubbling boron trifluoride gas into water until the molecular ratio of water to boron fluoride was approximately 1:1. The catalyst and toluene were placed in a flask and stirred while adding the olefin dropwise over an interval of 1.6 hours. The temperature rose from 40° C. to 53° C. Heating was continued for an additional hour. The catalyst was then removed and the catalyst-free reaction mixture was washed three times with water, dried, and freed of excess toluene. The dodecyl-toluene product was distilled at an absolute pressure of from 2 to 5 mm. Hg; at an overhead temperature of 156-170° C. The refractive index of the product at 20° C. was 1.4843.

The dodecyltoluene obtained was sulfonated by treating it with 1.5 parts by weight of fuming sulfuric acid (20 per cent  $\text{SO}_3$ ). The acid was added to the hydrocarbon while stirring and holding the temperature to 15-20° C. The reaction mixture was then warmed to 50° C. for five minutes. A small amount of water was added to the reaction mixture, causing the formation of a water phase and a hydrocarbon phase. The hydrocarbon phase was separated and dissolved in isopropyl alcohol containing 20 per cent water. An excess of solid guanidine carbonate was added causing the water to separate and to be basic to litmus. The alcohol fraction was separated, evaporated to dryness, redissolved in anhydrous isopropyl alcohol to separate any inorganic salts and again evaporated to dryness. The guanidine toluene sulfonate product was a firm glassy solid.

#### EXAMPLE II

Toluene was alkylated with hexadecene-1 by the procedure described in Example I. Reaction was less vigorous as heat had to be applied to maintain the reaction temperature at about 50° C. Total time of addition of olefin and heating was 5 hours. After excess toluene was removed by distillation hexadecyltoluene was recovered. The product boiled at 202-205° C. at an absolute pressure of from 4.5 to 4.8 mm. Hg. The hexadecyltoluene was sulfonated with fuming sulfuric acid and converted to guanidine sulfonate by saturating the isopropyl alcohol solution of the sulfonation mixture with guanidine carbonate. The solution was filtered and evaporated to dryness yielding the guanidine salt of hexadecyltoluene sulfonic acid.

#### EXAMPLE III

Toluene was alkylated with decene-1 by the previously described procedure. Decyltoluene was obtained having a boiling point of 138-141° C. at an absolute pressure of from 10-11 mm. Hg. The product was sulfonated and converted to the guanidine salt.

#### EXAMPLE IV

Benzene was alkylated with commercial isooctenes by the previously described procedure. The separated crude alkylate was distilled into a monoisoheptylbenzene fraction boiling from 98 to 113° C. at 9 mm. Hg. absolute pressure and a diisoheptylbenzene fraction boiling at 145-175° C. at 9 mm. Hg absolute pressure. The diisoheptyl fraction was sulfonated and converted to the guanidine salt.

#### EXAMPLE V

Diphenyl (Eastman White Label grade) was alkylated with tetradecene-1 using the general procedure described in Example I. In this case it was found desirable to omit the solvent during alkylation and to raise the temperature to 90° C. Benzene was added following the alkylation to facilitate the process of water washing. This benzene was removed by distillation and some unreacted diphenyl removed by filtration. A small amount of additional diphenyl was removed by distillation at 91-95° C. at 0.5 mm. Hg absolute. The tetradecyl diphenyl was distilled at 240-247° C. at 4 mm. Hg absolute pressure.

A portion of the above tetradecyl diphenyl was sulfonated and converted to the guanidine salt by the method described in Example I.

#### EXAMPLE VI

Naphthalene was alkylated with decene-1 by the procedure of Example I. The crude product was distilled obtaining 45 per cent of the material boiling at 195-200° C. at 5 mm. Hg absolute pressure which represented the monoalkylated naphthalene. This monoalkylated product was sulfonated and converted to the guanidine salt by the method of Example I.

#### EXAMPLE VII

Toluene was alkylated with a C<sub>8</sub> olefin fraction in the presence of anhydrous HF as a catalyst, at 100° F. Trihexyltoluene was recovered from the effluents of the reaction and when sulfonated, followed by neutralization of the resulting sulfonic acid with guanidine, is converted to guanidine trihexyltoluene sulfonate.

5  
EXAMPLE VIII

Topped Mid-Continent crude was distilled to produce two separate distillates corresponding to SAE 10 and 20 raw base stocks. The final distillation kettle product or vacuum reduced crude was then subjected to a two step solvent extraction employing liquid propane as the selective solvent. The propane extract of the first step contained oil of an average viscosity of about 100 SUS at 210° F. (SAE 50 base stock) and the propane extract of the second step contained oil of an average viscosity of about 220 SUS at 210° F. (SAE 250 base stock).

The raw SAE 250 base stock was recovered from the total extract of the second extraction step and then subjected to solvent extraction employing phenol as the selective solvent and to propane solvent dewaxing to produce a highly paraffinic raffinate comprising a lubricating oil stock having the following properties:

|                           |       |    |
|---------------------------|-------|----|
| Viscosity, SUS at 100° F. | 5313  | 20 |
| Viscosity, SUS at 210° F. | 223.3 |    |
| Viscosity index           | 89    |    |
| Gravity, °API at 60 F.    | 24    |    |
| Average molecular weight  | 730   |    |

A solution of 1000 grams of the lubricating oil stock described above dissolved in liquid ethylene chloride was slowly mixed with a solution of 176 grams of sulfur trioxide also dissolved in liquid ethylene chloride at a temperature maintained within the limits of 75 to 115° F. at atmospheric pressure, under which conditions reaction of sulfur trioxide with the lubricating oil began almost immediately to produce petroleum sulfonic acid. Reaction was completed shortly after admixing of the reactants was terminated.

To the resulting reaction mixture (including ethylene chloride) was added 103 grams of guanidine carbonate. The mixture was stirred vigorously at a temperature within the limits of 70 to 110° F., whereby the guanidine carbonate reacted with the acidic constituents to produce a mixture of guanidine petroleum sulfonates, guanidine sulfate, guanidine sulfite and traces of guanidine carboxylates. Ethylene chloride was then removed from the reaction mixture by vaporization.

The total reaction product, free of ethylene chloride, comprised guanidine petroleum sulfonates in oil solution and was admixed with an equal volume of anhydrous isopropyl alcohol with vigorous stirring, at a temperature near the boiling point of the alcohol at atmospheric pressure. Under these conditions the guanidine petroleum sulfonate reaction product and oil were dissolved in the alcohol. The alcohol mixture contained some suspended solids and was filtered at its existing temperature. The filtrate was permitted to cool to room temperature, and a large portion of the solute then separated therefrom, as a gummy viscous liquid. The cooled alcohol solution, i. e., at about 70° F., containing guanidine petroleum sulfonates not readily dispersible in oil was decanted from the separated viscous liquid, the latter comprising an oil solution or dispersion of oil-soluble guanidine petroleum sulfonates. The oil solution was then washed with alcohol at room temperature and the washings were added to the previously decanted liquid. The remaining alcohol was stripped from the gummy viscous liquid, and the liquid was purified, i. e., freed of occluded salts, by dissolving it in benzene, washing the benzene solution with water, and then stripping until the product was benzene-free. The purified product consisted of 600 grams of a dark brown, viscous oil solution of guanidine petroleum sulfonate, and is referred to hereinafter in this example as the "alcohol-insoluble product," i. e., insoluble at room temperature. Several properties of the alcohol-insoluble product are listed as follows:

|                            |        |
|----------------------------|--------|
| Specific gravity, 60/60 F. | 0.8887 |
| Gravity, °API at 60 F.     | 27.7   |
| Per cent nitrogen          | 1.08   |

Alcohol was stripped from the decanted alcohol solution described above. The remaining alcohol-free liquid was purified by dissolving it in toluene, water washing, and then stripping until free of toluene. Toluene was used in the purification of this liquid instead of benzene, in view of its higher boiling point, thus permitting a higher solu-

tion purification temperature for the guanidine petroleum sulfonates. The resulting purified guanidine petroleum sulfonates, soluble in isopropyl alcohol at 70° F., as compared with the alcohol-insoluble liquid described above, are referred to hereinafter in this example as "alcohol-soluble" guanidine petroleum sulfonate.

The alcohol-soluble and alcohol-insoluble guanidine petroleum sulfonates were each incorporated with separate portions of a lube oil base, and each resulting blend was tested in accordance with the NBS stability test (McKee and Fritz, "Analytical Chemistry" 21, 568, 1949). In carrying out this test, thermal stability of an oil, in this case a lubricating oil containing a guanidine petroleum sulfonate as an additive, is determined by passing it as a thin film over a steel strip under controlled temperature conditions, over a specified period, and the amount of any resulting deposition of degradation product on the strip is measured. Flat steel strips are employed. The tests conducted were modified in two particulars: (1) the steel strips were curved slightly upward at the edges to prevent the test oil from running off the sides, and (2) a single 12 hour period was used instead of the two 6 hour periods. Each product, i. e., the alcohol-soluble and the alcohol-insoluble guanidine petroleum sulfonate, was added to the base oil<sup>1</sup> in a concentration which yielded an oil-additive solution containing the same number of milli-equivalents of additive as does a 2 per cent solution of a commercially available detergent sold under the trade name of "Paranox 64" and comprising an alkaline earth metal salt of an alkylphenol sulfide. A blend of the same base oil with 4 volume per cent of Paranox 64 was tested in the same manner for comparison. The results of these thermal stability tests are summarized in the following tabulation:

| Material Tested                                                        | Deposit, mg. | Appearance of Strip |
|------------------------------------------------------------------------|--------------|---------------------|
| Base oil <sup>1</sup>                                                  | 90.6         | Poor.               |
| Base oil <sup>1</sup> +alcohol-soluble guanidine petroleum sulfonate   | 247          | Very poor.          |
| Base oil <sup>1</sup> +alcohol-insoluble guanidine petroleum sulfonate | 12.6         | Very good.          |
| Base oil <sup>1</sup> +4 percent Paranox 64                            | 9.8          | Do.                 |

<sup>1</sup> A solvent refined SAE 30 lubricating oil containing 0.75 volume percent of a commercially available oxidation inhibitor,  $\text{P}_2\text{S}_5$ -reacted terpenes.

<sup>2</sup> The alcohol-soluble guanidine petroleum sulfonate did not dissolve completely in the base oil.

The alcohol-insoluble guanidine petroleum sulfonate was evaluated as a lubricating oil additive by dissolving it in the base oil already described and then testing the resulting blend in a mounted single cylinder H2 Lauson test engine operated under conditions simulating the CRC L-4 test conditions. The test performed consists of placing 900 grams of the lubricating oil in the crankcase of the single cylinder engine, and operating the engine under a 1.2 H. P. load at  $1600 \pm 20$  R. P. M., while maintaining a cooling jacket temperature of 210° F., and oil temperature of 310° F., and an air to fuel ratio of 13.5:1. At the end of 60 hours operation under these conditions, the engine is stopped, disassembled, and the piston, crankcase, and bearings are examined. The piston varnish, crankcase, base sludge, overall varnish and carbon, and overall sludge are rated on an arbitrary scale of 1 to 10, the value 10 representing as nearly perfect as ascertainable, number 1 being "very poor" and numbers 2 to 9 each representing intermediate ratings. As a standard for further evaluation of the blend of lubricating oil and alcohol-insoluble guanidine petroleum sulfonate, the same base oil, but without added guanidine petroleum sulfonate, was tested in exactly the same manner. The base oil blend tested contained the same per cent by weight of the alcohol-insoluble guanidine petroleum sulfonate as used in the strip test described in the foregoing paragraph. For a further comparison, a blend of the same base oil with 4.4 volume per cent of a commercially available oil detergent sold as Lubrizol 67 and comprising a barium petroleum sulfonate was tested in the Lauson engine, in the same manner. This latter blend of base oil with Lubrizol 67 contained the same number of equivalents of sulfonate groups as the tested blend containing guanidine

## EXAMPLE XI

An additional portion of the isopropyl alcohol-insoluble sodium petroleum sulfonate prepared as described in Example X was treated in the same manner as in Example X except that barium chloride was substituted for guanidine carbonate. The resulting reaction product was analyzed for sulfated ash. The sulfated ash formed was leached with water to remove water-soluble ash. The total sulfated ash content was 18.2 per cent and the water-insoluble sulfated ash content was only 1.6, thus indicating that the alcohol-insoluble sodium petroleum sulfonate was substantially unreactive to form the barium salt. These data further distinguish the commercially available sodium petroleum sulfonates from the sodium petroleum sulfonates of Example X inasmuch as that material can be converted to the barium salt by the method of this example.

7 petroleum sulfonate. The following is a tabulation of the results of the Lauson type engine test described:

|                            | Base oil <sup>1</sup> | Base oil <sup>1</sup> + alcohol-insoluble guanidine petroleum sulfonate <sup>2</sup> | Base oil <sup>1</sup> + alcohol-insoluble guanidine petroleum sulfonate <sup>3</sup> | Base oil <sup>1</sup> + 4.4 volume per cent Lubrizol 67 <sup>4</sup> |
|----------------------------|-----------------------|--------------------------------------------------------------------------------------|--------------------------------------------------------------------------------------|----------------------------------------------------------------------|
| Piston varnish             | 5.0                   | 9.0                                                                                  | 9.8                                                                                  | 9.0                                                                  |
| Crankcase and base sludge  | 6.2                   | 8.2                                                                                  | 8.8                                                                                  | 8.8                                                                  |
| Overall sludge             | 7.0                   | 8.5                                                                                  | 8.9                                                                                  | 8.8                                                                  |
| Overall varnish and carbon | 6.3                   | 8.4                                                                                  | 9.3                                                                                  | 8.6                                                                  |
| Ring sticking              | 10.0                  | 10.0                                                                                 | 10.0                                                                                 | 9.0                                                                  |
| Bearing weight loss, mg.   | 12.1                  | 3.8                                                                                  | 7.3                                                                                  | 4.6                                                                  |

<sup>1</sup> Solvent refined SAE 30 lubricating oil, containing 0.75 volume per cent of a commercially available oxidation inhibitor comprising  $P_2S_4$ —reacted terpenes.

<sup>2</sup> This blend contains an amount of Lubrizol 67 in a concentration equivalent to the number of active detergent groups in an oil containing 2 volume per cent Paraxon.

<sup>3</sup> This blend contains an amount of alcohol-insoluble guanidine petroleum sulfonate in a concentration equivalent to the number of active detergent groups in an oil containing 4 volume per cent Paraxon 64.

<sup>4</sup> This blend contains an amount of alcohol-insoluble guanidine petroleum sulfonate in a concentration equivalent to the number of active detergent groups in an oil containing 2 volume per cent Paraxon 64.

The data listed in the preceding tabulation clearly illustrate that the ash-free guanidine petroleum sulfonates of our invention are comparable in effectiveness with well established commercial metal-containing detergents.

## EXAMPLE IX

A water solution containing guanidine carbonate in slight excess of that required to react with sodium petroleum sulfonate was added with agitation to an aqueous dispersion of a commercially available sodium petroleum sulfonate maintained at 70° F. Under these conditions the sodium petroleum sulfonate reacted with the guanidine carbonate to form a firm plastic mass which separated from the resulting reaction mixture, and which upon cooling formed a gel that while suitable as a grease was not suitable for use as an oil detergent. This reaction demonstrates that a guanidine petroleum sulfonate detergent material of our invention cannot be prepared merely by reacting a commercially available petroleum sulfonic acid or a salt thereof, with a guanidine salt such as guanidine carbonate. Further, it demonstrates the commercially available sodium petroleum sulfonate to be sufficiently water-soluble to be reactive in aqueous medium with guanidine carbonate.

## EXAMPLE X

The SAE 250 lube oil stock of Example VIII was sulfonated in accordance with the procedure of Example VIII. The petroleum sulfonic acid product was then converted to a sodium salt by neutralization with sodium hydroxide, and the total resulting neutralization product was subjected to solvent extraction with isopropyl alcohol at room temperature. A portion of a resulting alcohol-insoluble sodium salt thus formed, was treated with aqueous guanidine carbonate in accordance with the procedure of Example IX. No reaction appeared to take place and the sodium sulfonate layer was separated from the aqueous guanidine carbonate layer and then contacted with a fresh aqueous guanidine carbonate solution. The sulfonate layer was again separated and water washing was attempted but resulted in formation of a stable emulsion. A sample of the sulfonate layer upon analysis for nitrogen was found to contain 0.55 per cent nitrogen. The sulfated ash content of the sulfonate product was determined and was found to be 4.68 per cent, indicating a high sodium content. These two analytical results indicate that the sodium petroleum sulfonate of this example was substantially unreacted with the guanidine carbonate. In this regard the sodium petroleum sulfonate prepared from the SAE 250 oil, as already described in this example, differs markedly from the commercially available petroleum sodium sulfonate of Example IX, inasmuch as in the present example the sodium petroleum sulfonate is too insoluble in water to be reacted with the aqueous guanidine carbonate, whereas the commercially available sodium petroleum sulfonate was sufficiently soluble in water so as to be reacted with guanidine carbonate.

20

Listed as oil compositions I-V in the following tabulation are several lube oil blends and also a base oil free of any additive material, each of which was evaluated in a series of Lauson engine tests of the type described in Example VIII. These evaluation tests are summarized as follows:

|    |                                                      | Composition |       |      |       |       |
|----|------------------------------------------------------|-------------|-------|------|-------|-------|
|    |                                                      | I           | II    | III  | IV    | V     |
| 30 | Lubricating Oil, volume percent                      | 100.0       | 99.25 | 99.0 | 94.75 | 94.50 |
|    | Oxidation Inhibitor, <sup>1</sup> volume percent     | 0.0         | 0.75  | 0.5  | 0.75  | 1.00  |
| 35 | Guanidine octadecyltoluene sulfonate, weight percent | 0.0         | 0.0   | 0.5  | 0.0   | 0.0   |
|    | U. B. Bray Detergent, weight percent                 | 0.0         | 0.0   | 0.0  | 4.5   | 4.5   |

<sup>1</sup> Commercially available ( $P_2S_4$ —reacted terpenes) oxidation inhibitor.

40

The oil employed as the base oil in these compositions was a solvent refined Mid-Continent oil of lubricating grade having the following characteristics:

|                     |          |
|---------------------|----------|
| Gravity API         | 30.3     |
| Viscosity at 210° F | 61.8 SUS |
| Viscosity index     | 98       |
| Neutralization No.  | 0.01     |

|    |                                   | Rating of Composition<br>(Evaluation Scale, 1-10) |     |     |     |     |
|----|-----------------------------------|---------------------------------------------------|-----|-----|-----|-----|
|    |                                   | I                                                 | II  | III | IV  | V   |
| 55 | Piston Varnish Rating             | 9.2                                               | 7.9 | 8.4 | 9.8 | 9.5 |
|    | Crankcase and base sludge rating  | 9.0                                               | 8.6 | 8.2 | 8.0 | 9.3 |
|    | Overall varnish and carbon rating |                                                   |     | 8.4 |     |     |
|    | Overall sludge rating             |                                                   |     | 8.7 |     |     |
|    | Bearing weight loss, mg.          | 1,098                                             | 6.5 | 1.2 | 201 | 180 |

60

The data of Example XII illustrate the base oil alone to exhibit desirable piston varnish ratings and crankcase and base sludge ratings. However use of the base oil alone results in high bearing weight loss. Accordingly an oxidation inhibitor is employed as illustrated in column II for the purpose of reducing bearing weight loss. The use of such an inhibitor effectively reduces piston varnish rating, and crankcase and base sludge rating. Guanidine octadecyltoluene sulfonate, although it contains only 26 carbon atoms in the molecule and is for that reason less desirable than are other oil detergents having a larger number of carbon atoms in the molecule, provides an improvement in the bearing weight loss and in the varnish rating of the base oil tested.

70

The data of Example XII further illustrate the improvement of guanidine-octadecyltoluene sulfonate over a commercial additive marketed by the U. B. Bray Company particularly in regard to bearing weight loss.

80

EXAMPLE XIII

A guanidine petroleum sulfonate detergent was prepared substantially in accordance with the procedure outlined hereinbefore. The petroleum sulfonation stock was the same as described in Example VIII. Batch sulfonation was carried out in a stainless steel vessel by slowly adding with agitation 450 grams of  $SO_2$ , stabilized

against polymerization, and dissolved in 2000 grams of ethylene chloride, to 4000 grams of oil dissolved in 3000 grams of ethylene chloride. The sulfonation temperature was maintained at 70° F. throughout the reaction. The reaction mixture was immediately neutralized by stirring in 700 grams of commercial guanidine carbonated in the form of an aqueous slurry. The neutralized reaction mixture was washed four times with water using one volume of wash water per volume of total reaction mixture per wash. The ethylene chloride solvent was evaporated from the water-washed product and separation of undesirable guanidine sulfonates was effected by multiple batch extraction with isopropyl alcohol. Four batch extractions were carried out using 2 volumes of the alcohol per volume of hydrocarbon phase in the first extraction and 3/4 volume of alcohol in the subsequent extractions. After evaporation of isopropyl alcohol from the final extraction residue the yield of guanidine petroleum sulfonates plus unreacted oil amounted to 2500 grams. The total nitrogen content of this concentrate was 0.96 per cent by weight which indicates a guanidine petroleum sulfonate content of about 20 per cent by weight.

For purposes of engine evaluation 21.4 weight per cent of the above concentrate was added to a base oil, the same as that of Example VIII, which contains the oxidation inhibitor primarily to provide bearing protection for the test engine. Expressed as the number of ionic weight equivalents the preceding blend provides a concentration of guanidine and sulfonate groups exactly equal to that of the barium and phenate groups contained in a 4 volume per cent concentration of the commercial detergent "Paranox 64" in the same base oil, also containing 0.75 volume per cent of the oxidation inhibitor. The two test oils, therefore, were exactly equivalent insofar as concentration of surface active groups are concerned; i. e., two sulfonate molecules per one "Paranox 64" molecule since the latter contains 2 active phenolic groups per molecule.

Parallel engine tests were completed on both of the above oils using a modified H2-Lauson engine operating under severe conditions simulating the CRC L-1 diesel engine test for lube oil detergents. The essential test difference between these tests and those of Example VIII are: oil temperature 225° F. and jacket temperature, 300° F. On completion of the tests, the engines were rated as described in Example VIII to give the following results:

|                                 | Base oil <sup>1</sup> +<br>oil-soluble<br>guanidine<br>petroleum<br>sulfonate | Base oil <sup>1</sup> +<br>4 volume<br>per cent<br>Paranox 64 |
|---------------------------------|-------------------------------------------------------------------------------|---------------------------------------------------------------|
| Piston varnish.....             | 7.4                                                                           | 7.7                                                           |
| Crankcase and base sludge.....  | 8.5                                                                           | 9.2                                                           |
| Overall sludge.....             | 8.6                                                                           | 9.2                                                           |
| Overall varnish and carbon..... | 7.1                                                                           | 7.1                                                           |
| Oil ring plugging.....          | 9.8                                                                           | 9.0                                                           |
| Ring sticking.....              | 6.7                                                                           | 10.0                                                          |
| Bearing weight loss, mg.....    | 6.3                                                                           | 10.5                                                          |

<sup>1</sup> The same as employed in Example VIII.

The above results are especially significant inasmuch as Paranox 64 is a qualified diesel oil detergent capable of passing the stringent L-1 test. The only unfavorable comparison between the two additives is that of ring sticking where the actual difference was not as pronounced as the rating would indicate.

#### EXAMPLE XIV

10 Table 1 gives the physical properties of the white mineral oil used in the preparation and attempted preparation of greases as shown in Table 2.

15 Table 2 shows clearly how the alkyl aryl sulfonates of the metals ordinarily used in grease making did not form the proper gels under similar conditions as did the corresponding sulfonates of guanidine. Listed across the top of the table are the various aromatics and olefins with which they were alkylated. After alkylation, each alkyl aromatic was sulfonated and then neutralized to form the salt of the element or compound in the left-hand vertical column. In each column beneath the particular alkyl aromatic indicated are the results of attempting to form a grease with the mineral oil described in Table 1.

20 Table 3 indicates the micropenetration of two of the better greases, those formed with guanidine dodecyltoluene-sulfonate and guanidine hexadecyltoluene sulfonate, shown in Table 2, per indicated strokes of a grease worker. The test method used for determining the micropenetration of the grease is that of the American Society for Testing Materials and is designated as ASTM, D 217-47T, as modified according to "Industrial and Engineering Chemistry," Analytical edition, vol. 11, pp. 108-110 (1939). The micropenetration is the distance, measured in tenths of a millimeter, which the cone penetrates the grease in 5 seconds. According to this method, an ASTM penetrometer is used with a modified cone weighing 20 grams. The grease of which the penetration is to be measured is put in the grease container holding about 3 to 5 grams and the top surface leveled off. The container is then placed on the penetrometer base and tested. The grease worker referred to above is also described in the indicated ASTM test method. It briefly comprises a cup with a top for closing through which extends a plunger. Attached to the plunger is a perforated plate which, when the grease worker is in operation, passes back and forth forcing the grease in the cup to pass through the perforations.

25 Table 4 shows the decrease in the micropenetration for guanidine dodecyltoluene sulfonate grease, for which the micropenetrations per indicated strokes in the grease worker are shown in Table 3, after sitting undisturbed for the times indicated.

30 *Table 1.—Characteristics of white mineral oil used*

|                                                      |        |
|------------------------------------------------------|--------|
| Viscosity at 100° F. SUS.....                        | 183.2  |
| Viscosity at 210° F. SUS.....                        | 44.92  |
| Viscosity index.....                                 | 90.0   |
| Refractive index, N <sub>D</sub> <sup>20</sup> ..... | 1.4748 |
| Specific gravity, D <sub>420</sub> .....             | 0.8690 |
| Specific dispersion.....                             | 102    |

35 *Table 2*

| Radical With<br>Which Salt Is<br>Formed | Hydrocarbon Group                 |                              |                            |                            |                            |
|-----------------------------------------|-----------------------------------|------------------------------|----------------------------|----------------------------|----------------------------|
|                                         | Methylbutene<br>+Benzene          | Octene-1<br>+Toluene         | Decene-1<br>+Toluene       | Dodecene-1<br>+Toluene     | Hexadecene-1<br>+Toluene   |
| Lithium.....                            | Soft Plastic Mass,<br>Slight gel. | Soluble in Oil, No<br>gel.   | Soluble in Oil, No<br>gel. | .....                      | .....                      |
| Sodium.....                             | Insoluble in Oil.....             | Slight gel.....              | .....                      | Soluble in Oil, No<br>gel. | Soluble in Oil, No<br>gel. |
| Potassium.....                          | .....                             | .....                        | .....                      | .....                      | Do.                        |
| Calcium.....                            | Insoluble in Oil,<br>Waxy Solid.  | Soluble in Oil, No<br>gel.   | Soluble in Oil, No<br>gel. | .....                      | Slight gel.                |
| Strontium.....                          | .....                             | do.....                      | .....                      | Soluble in Oil, No<br>gel. | Weak gel.                  |
| Barium.....                             | .....                             | Very weak gel.....           | Weak gel.....              | Weak gel.....              | Weak gel.                  |
| Guanidine.....                          | Insoluble in Oil, No<br>gel.      | Insoluble in Oil,<br>No gel. | Fair Grease.....           | Good Grease.....           | Good Grease.               |

Table 3.—Work stability

|                                             | Micropenetration at Indicated Working Strokes |    |       |       |        |        |         |
|---------------------------------------------|-----------------------------------------------|----|-------|-------|--------|--------|---------|
|                                             | 1                                             | 60 | 1,000 | 5,000 | 10,000 | 20,000 | 100,000 |
| Guanidine Dodecyltoluene Sulfonate Grease   | 46                                            | 59 | 75    | 75    | 86     | 147    |         |
| Guanidine Hexadecyltoluene Sulfonate Grease | 45                                            | 45 | 62    | 82    | 91     | 115    | 177     |

Table 4.—Reversion of guanidine dodecyltoluene sulfonate worked 100,000 times

| Total Time of Sitting Undisturbed at Room Temperature in Hours | Micropenetration |
|----------------------------------------------------------------|------------------|
| 0                                                              | 147              |
| 1.0                                                            | 71               |
| 3.5                                                            | 55               |
| 6.0                                                            | 49               |
| 20.0                                                           | 43               |
| 48.0                                                           | 40               |

## EXAMPLE XV

This example shows another great advantage of our invention, that of utilizing a mixture of olefins for alkylating the aromatic. In this instance, a fraction of cracked naphtha boiling in the range of 246 to 260° C. and containing only 40 per cent olefins was used to alkylate toluene. This product was sulfonated and then neutralized with guanidine carbonate. The olefins, some of which were branched, had the double bond in various positions in addition to the 1-position. Thus, it is shown that our invention may be practiced successfully using easily obtained refinery cuts without extensive purification.

The grease was made by dispersing 20 parts by weight of the guanidine sulfonate in 80 parts by weight of the mineral oil by heating to a temperature of between 200 and 240° C. and then cooling. The resulting gel was then milled to a smooth grease.

Table 1 gives the physical properties of the mineral oil used to form the grease with the guanidine alkyl aryl sulfonate.

In Table 5 the micropenetration of the grease prepared as described above is compared with that of three commercial all-purpose greases purchased on the open market. Grease A was a barium base grease made from lube oil in which the gelation agent was derived from fatty acids. Grease B was a lithium base grease having the gelation agent made by treating fatty acids. Commercial grease C is a sodium base grease of which the gelation agent was made by saponifying nonedible tallow with sodium hydroxide. As may be observed, our grease is equal to or better than the comparative greases. Note that commercial grease B exceeded a penetration of 420, which is about the maximum measuring limit of the penetrometer, after only 10,000 strokes in the grease worker.

Table 5.—Work stability

|                                       | Micropenetration at Indicated Working Strokes |     |       |       |        |        |         | Change in Micropenetration between 1,000 and 100,000 strokes | Percent Change in Micropenetration between 1,000 and 100,000 strokes |
|---------------------------------------|-----------------------------------------------|-----|-------|-------|--------|--------|---------|--------------------------------------------------------------|----------------------------------------------------------------------|
|                                       | 1                                             | 60  | 1,000 | 5,000 | 10,000 | 50,000 | 100,000 |                                                              |                                                                      |
| Guanidine Alkyl Aryl Sulfonate Grease | 27                                            | 52  | 70    | 93    | 94     | 122    | 146     | 67                                                           | 85                                                                   |
| Commercial Grease A                   | 125                                           | 124 | 145   | 175   | 192    | 244    | 269     | 124                                                          | 86                                                                   |
| Commercial Grease B                   | 158                                           | 193 | 275   | 380   | 420    | —      | —       | above 145 at 10,000                                          | above 52 at 10,000                                                   |
| Commercial Grease C                   | 53                                            | 73  | 107   | 137   | 151    | 199    | 237     | 127                                                          | 119                                                                  |

## EXAMPLE XVI

A soft grease was made by using the guanidine salt of an alkyl aryl sulfonic acid in which the olefins used in producing the alkyl aromatic boiled in the range of 190° to 200° C., and the aromatic was toluene. Only a small portion of the thus formed soap or gelation agent dispersed in the mineral oil used; however, the portion which did, produced a satisfactory soft grease.

75 as their metal salts, in a mineral oil. A mineral oil similar to those used in the previous examples was used here.

Table 8

| 80                       | Salt | Solubility in Oil                      |
|--------------------------|------|----------------------------------------|
| Guanidine laurate        | —    | Insoluble, stratified on cooling.      |
| Guanidine stearate       | —    | Hard waxy cake, worked to poor grease. |
| Phenylbiguanide carotate | —    | Poor grease.                           |

**13**  
**EXAMPLE XX**

An SAE 250 oil of the type described in Example VIII was sulfonated, neutralized with guanidine carbonate, water washed, and alcohol extracted, in accordance with the procedure of Example VIII. The alcohol soluble portion was stripped of alcohol and dissolved in hot methylisobutyl ketone. On cooling, a precipitate of diguanidine disulfonate crystallized and was separated by suction filtration. The solid was washed with a small amount of cold methylisobutyl ketone, and then recrystallized from ketone. Analysis of the original charge oil and the disulfonate are given in the following table along with formulas calculated from these analyses.

| Charge<br>Oil,<br>Found | Diguanidine Disulfonate         |                                                                                |
|-------------------------|---------------------------------|--------------------------------------------------------------------------------|
|                         | Found                           | Calculated                                                                     |
| C-----                  | 85.69                           | 65.6                                                                           |
| H-----                  | 12.84                           | 9.7                                                                            |
| S-----                  |                                 | 6.2                                                                            |
| N-----                  |                                 | 8.2                                                                            |
| O-----                  |                                 | * 10.3                                                                         |
| Mol Wt.                 | 730                             | 1,050                                                                          |
| Formula.....            | C <sub>12</sub> H <sub>14</sub> | b C <sub>12</sub> H <sub>14</sub> S <sub>2</sub> N <sub>2</sub> O <sub>4</sub> |

\* By difference.

† Based on formula of charge oil.

The diguanidine disulfonate thus produced was dissolved in hot oil; the resulting oil-diguanidine disulfonated mixture became a grease upon cooling.

As will be evident to those skilled in the art, various modifications can be made or followed, in the light of the foregoing disclosure and discussion, without departing from the spirit or scope of the disclosure or from the scope of the claims.

We claim:

1. As a new class of compositions, synthetic guanidine alkyl hydrocarbonaryl sulfonates containing a total number of at least 10 carbon atoms in the alkyl groups.

2. As a new class of chemical compounds, the guanidine salts of alkyl hydrocarbonaryl sulfonic acids having a total number of carbon atoms in the alkyl groups in the range of 10 to 20.

3. As a new class of chemical compounds, the guanidine salts of alkyl hydrocarbonaryl sulfonic acids having a total number of carbon atoms in the alkyl groups in the range of 10 to 20, having at least one alkyl group containing at least 10 carbon atoms, and having the property of forming lubricants when dispersed in mineral oil.

4. A new class of chemical compounds according to claim 3 wherein the aryl nucleus is selected from the group consisting of benzene, naphthalene, diphenyl, anthracene, and their lower alkyl homologues.

5. As a new class of chemical compounds, the guanidine salts of alkyl hydrocarbonaryl sulfonic acids having a total number of carbon atoms in the alkyl groups of not more than 20, having at least two alkyl groups of at least 8 carbon atoms each, and having the property of forming a lubricant when dispersed in mineral oil, wherein the aryl nucleus is selected from the group consisting of benzene, naphthalene, diphenyl, anthracene, and their lower alkyl homologues.

6. As a new chemical compound, guanidine dodecyltoluene sulfonate.

**14**

7. As a new chemical compound, guanidine hexadecyltoluene sulfonate.

8. A guanidine alkyl hydrocarbonaryl sulfonate containing at least 10 alkyl carbon atoms and not more than 35 carbon atoms in the molecule.

9. A process for the manufacture of a guanidine alkyl aryl sulfonate suitable as a lubricant component, comprising sulfonating a synthetic alkyl aromatic hydrocarbon containing at least 10 alkyl group carbon atoms in the molecule, neutralizing sulfonic acid thus produced with a guanidine compound selected from the group consisting of guanidine and a basic guanidine salt, resulting neutralization product containing a guanidine alkyl aryl sulfonate of at least one of the group consisting of oil-soluble and oil-insoluble guanidine alkyl aryl sulfonates, separating one of said oil-soluble and oil-insoluble guanidine alkyl sulfonates from any of the other in said neutralization product, and recovering at least one of said oil-soluble and oil-insoluble sulfonates thus separated, as product of the process.

10. The process of claim 9 wherein an oil-soluble guanidine alkyl aryl sulfonate is recovered as said product.

11. The process of claim 9 wherein an oil-insoluble guanidine alkyl aryl sulfonate is recovered as said product.

12. The process of claim 10 wherein said oil-soluble guanidine sulfonate contains from 40-70 carbon atoms in the molecule.

13. The process of claim 10 wherein said oil-soluble guanidine sulfonate contains from 24-34 carbon atoms in the molecule.

14. The process of claim 11 wherein said oil-insoluble sulfonate contains from 17-35 carbon atoms in the molecule.

15. The process of claim 9 wherein oil-soluble and oil-insoluble sulfonates are separated by alcohol extraction.

16. The process of claim 11 wherein said alkyl aromatic hydrocarbon to be sulfonated, is a product of alkylation of an aromatic hydrocarbon with an olefin fraction boiling in the range of 190-350° F.

17. As a new class of chemical compounds, the guanidine salts of alkyl aryl sulfonic acids wherein the aryl nucleus is selected from the group consisting of benzene, naphthalene, diphenyl, anthracene, and their lower alkyl homologues, having a total number of carbon atoms in the alkyl groups of not more than 20, having at least three alkyl groups of at least 6 carbon atoms each, and having the property of forming a lubricant when dispersed in mineral oil.

18. As a new chemical compound, guanidine trihexyltoluene sulfonate.

19. A guanidine alkyl hydrocarbonaryl sulfonate containing from 40 to 70 carbon atoms in the molecule.

20. As a new chemical compound, guanidine decyl-naphthalene sulfonate.

21. As a new chemical compound, guanidine tetradecyl diphenyl sulfonate.

**References Cited in the file of this patent**

**UNITED STATES PATENTS**

|           |                |               |
|-----------|----------------|---------------|
| 2,061,601 | Steik          | Nov. 24, 1936 |
| 2,076,623 | De Groote      | Apr. 13, 1937 |
| 2,223,935 | Daniels et al. | Dec. 3, 1940  |
| 2,473,112 | Short          | June 14, 1949 |